

Patented Aug. 2, 1927.

1,638,001

# UNITED STATES PATENT OFFICE.

HARRY E. BROOKBY, OF EVANSTON, ILLINOIS, ASSIGNOR TO UNITED STATES GYPSUM COMPANY, OF CHICAGO, ILLINOIS, A CORPORATION OF ILLINOIS.

## LIGHT-WEIGHT GYPSUM PRODUCT.

No Drawing.

Application filed August 19, 1922. Serial No. 583,040.

This invention relates to improvements in building material and more particularly to the production of a light weight plaster board and the method of making same.

5 Plaster board having a plaster body with fibrous cover sheets adhering to the flat faces has been used for a long time in the building trade as a substitute for wooden or metal lath and more recently the improvements 10 in plaster board have produced a plaster wallboard which in effect is a factory made plaster wall and there is a demand all over the country for the plaster wallboard that when nailed to the studding of the building 15 is ready for decoration and which provides a fireproof wall that remains uniform under all changes in temperature or atmospheric conditions, that is, it does not warp or buckle nor does it shrink or crack after it 20 has been erected.

This plaster board and plaster wallboard is made in standard widths and thicknesses and cut in desired lengths and weighs between 1,850 and 2,000 pounds per thousand 25 square feet. The gypsum from which these boards are made is a natural deposit and is found only in certain sections of this country and, on account of the nature of the mineral, plaster board plants are usually located at or near the gypsum mines with the result that it is necessary to transport the plaster board great distances to supply the demand in territories where there are no gypsum deposits and on account of the 30 weight increases the cost considerable to the users in such territories.

It is an object of this invention to reduce the weight of the plaster body of plaster board and wallboard while at the same time 40 maintaining the other high standardized qualities. The commercial advantages of such an improvement are obvious as well as the advantage to the purchasing public.

Since this invention relates to the composition of the body of the plaster board and may be applied to any of the well known 45 plaster boards now on the market which are universally produced by well known machines in which a fibrous cover sheet is advanced, the plaster body in a plastic state 50 deposited upon the advancing cover sheet, a top fibrous cover sheet applied over the plastic mass and the two cover sheets with the plastic body passed through a board

forming device comprising a pressure roller 55 that imparts the desired thickness to the board and then carried in a continuous strip upon a conveyor a great enough distance to allow the plastic body to set sufficiently to be cut into the desired lengths at the 60 end of the conveyor, removed and transported to the drying kilns, it is not necessary to illustrate or describe such a machine in more specific detail, yet it is to be understood that minor detail changes, such as in 65 the preferred proportions of the ingredients employed in carrying out this invention, may be made without departing from the scope thereof.

The plastic mass forming the plastic body 70 deposited upon the cover sheet as above described is calcined gypsum, or plaster of Paris, mixed with water and usually wood fibre or other aggregate, generally mechanically mixed on the conveyor that deposits 75 it. In accordance with this invention a certain proportion of a stock solution of casein dissolved in water and ammonium hydroxide, is incorporated during the mixing of the plastic mass forming the body of 80 the board. The casein solution forms a voluminous suspension compound with the calcined gypsum plastic mix while the ammonia used for the casein solution becomes ammonium sulphate, which is an inert substance. The gypsum casein compound is quite extended and voluminous and, in suspension, displaces a corresponding volume 85 of the heavier plastic calcined gypsum. In other words, the mixture at this stage substantially comprises, on the one hand, a large number of suspended dispersed gelatinous particles of the gypsum-casein reaction product, and, on the other hand, suspended particles of plaster of Paris. When using 90 casein in the proportion hereinafter specified and in the manner described, the plaster board formed as a result of the bulkier mass of the gypsum casein compound is 20 to 25 per cent lighter in weight than 95 the usual plaster board, and is more pliable than if the casein had not been employed.

The stock solution is preferably made by first soaking commercial granulated casein in water, in the proportion of about 5 to 6 100 ounces of casein to the gallon of water, for approximately one hour with the water near the boiling point, which softens the casein,

after which one quarter to one half ounce of strong liquid ammonium hydroxide for each 5 to 6 ounces of casein is added and stirred until the casein goes into clear solution.

- 5 It is preferable, in order to keep the wall board safely pliable, to add to the mix of calcined gypsum, water and aggregate on the mixing and conveying belt before depositing on the board forming machine the above described casein stock solution. I have found that very satisfactory results may be obtained by using substantially one-half ounce of casein to ten square feet of 10 wall board or 0.33 cu. ft. of core volume of wall board. As casein compounds have a tendency to retard the set of calcined gypsum with water it is preferable to add a positive accelerator, such as commonly used 15 for this purpose, to avoid slowing down the board production.

The improved board made with this type of body is very strong due to the increased strength imparted to the porous body by the 20 cementing action of the calcium-casein compound, and is about 25 per cent lighter in weight per square foot than the ordinary gypsum boards of similar thickness, weighing between 1250 to 1350 pounds per thousand 25 square feet. By regulating or varying the amount of casein solution added to the mixture, and thereby controlling the amount of gypsum casein suspension compound, the weight of the board can be varied to meet 30 the desired structural and shipping conditions.

The body of calcined gypsum mixed with calcium caseinate bonds the fibrous cover sheets to it as well in the calcined gypsum 35 boards and such boards when dried is more water resistant than the ordinary gypsum board. While I have described my invention in connection with the production of light-weight plaster board, it is obvious that 40 it is equally applicable to the preparation of other light weight gypsum products such as tile, blocks and other cast or molded gypsum articles.

The application of this invention to a 45 gypsum block or tile is described in my co-pending application Serial No. 584,342, filed August 25, 1922.

Having thus described one method of successfully carrying out my invention, and 50 without limiting myself to the precise procedure herein disclosed, what I claim as

new and desire to be protected by Letters Patent of the United States is:

1. A dried light-weight cellular gypsum product comprising hydrated plaster of Paris as the major ingredient, and voids left by the contraction and drying of calcium caseinate contained therein.

2. A dried light-weight cellular gypsum product comprising hydrated plaster of Paris as the major ingredient, and voids produced by the contraction and drying of a gypsum and casein reaction product produced in said mass.

3. A light-weight cellular product comprising set plaster of Paris as the major ingredient and the dried reaction product of calcined hydrated gypsum and casein in solution, the casein being present in the proportion of substantially one-half ounce to substantially 0.33 cu. ft. of the entire product.

4. The method of producing numerous small voids in a set plaster of Paris product which comprises adding to a slurry of calcined gypsum and water an aqueous solution of ammonium caseinate in such an amount that voids will be formed when allowing the mass to set, harden and dry.

5. The process of producing a dried light-weight gypsum product which comprises making a plastic mass of calcined gypsum and water as the major ingredient, then producing a suspension of a gypsum casein reaction compound therein by adding to said major ingredient an aqueous solution of casein thus forming a composite mass which is allowed to set, harden and dry, the said casein solution being added in such reacting proportions with the major ingredient that a multitude of small dispersed voids results during the drying process and remain in the finished gypsum product.

6. The process of producing a light weight gypsum product which comprises making a plastic mass of calcined gypsum and water, then precipitating calcium caseinate therein by adding to said plastic calcined gypsum mass an aqueous solution of casein and ammonium hydroxide, said casein solution being proportioned substantially at the rate of one-half ounce of casein to substantially 0.33 cu. ft. of the composite mass, and then permitting the mass to set, harden and dry.

HARRY E. BROOKBY.